

## UNITED STATES PATENT OFFICE

2,089,587

## DENTURE

Enrique G. Touceda, Albany, N. Y., assignor to  
 Consolidated Car-Heating Company, Inc., Albany, N. Y., a corporation of New York

No Drawing. Application November 27, 1936,  
 Serial No. 112,983

## 4 Claims. (Cl. 32—2)

My invention relates to prosthetic articles and particularly to dentures and the like formed from metal, and preferably but not necessarily, by the process of casting.

5 In the making of dentures by casting, it is usual to take an impression in plastic material of the interior mouth and jaw structure. This reproduces exactly, in the plastic, all of the small irregularities of the mouth and jaw structure 10 and is used in making a pattern from which the denture is cast from a suitable metal or alloy.

In order exactly to reproduce in the cast article all the minute structural irregularities in the pattern, the metal used must have many 15 peculiar characteristics among which the following are of paramount importance: It must be highly fluent at casting temperatures because if it is viscous or sluggish when molten it will not run freely into the finer details of the mold. 20 This is particularly true where a skeleton bridge, plate or other structure having finely attenuated portions is being cast, but it is also true in the casting of full or partial plates of paper thickness where it is necessary to produce an article 25 conforming exactly to all of the finer rugae of the patient's mouth.

The metal, in the "as cast" condition, must have a clean surface so that grinding and polishing is substantially unnecessary or at least is reduced to an absolute minimum. Since the exterior surface of the denture, as cast, conforms 30 to the irregularities of the pattern and since many of these are of an extremely delicate nature, the removal of any substantial portion of 35 the surface of the casting destroys the fit thereof.

The metal used must be such that the shrinkage of the casting on cooling is extremely small otherwise it is impossible to obtain a cast denture which fits properly due to the impossibility, 40 arising from the particular nature of the pattern and the manner in which it is produced, of making substantial allowances for shrinkage. The metal must be tasteless. That is to say, 45 it must not have a disagreeable metallic taste. Furthermore, since it is to be used in the mouth, it must be resistant to corrosion and particularly resistant to the corrosive action of the ordinary food acids and particularly to lactic 50 acid which is invariably present in the mouth.

The metal must be strong, hard and highly 55 resistant to deformation even in attenuated sections. Yet, on the other hand, it must be capable of being bent to a considerable degree without fracture in order that bridges, clasps

and the like may be properly fitted. The yield point must be comparatively high in order that dentures made therefrom may be subjected to the distortion necessary in close and proper fitting without producing permanent deformation.

The melting point should be as low as possible not only to minimize the cost and the natural difficulties encountered in casting metals or alloys having extremely high melting points, but 10 also to minimize shrinkage on cooling; and the specific gravity of the composition should also be as low as possible in order that the dentures may be light in weight.

An alloy comprising principally nickel and 15 chromium and containing by weight from 65% to 90% of nickel and from 5% to 30% of chromium affords excellent possibilities for use in making dentures because of its cost as compared with the precious metals and also because of its high 20 resistance to the corrosive agents ordinarily encountered by dentures. However, such a composition is quite soft, the melting point is extremely high, and the alloy when molten is so 25 viscous that it is impossible to cast thin sections therefrom. Moreover, the surface of the alloy in the "as cast" condition is not suitable 30 for dentures because of the dirt and scale which must be removed therefrom by grinding and polishing.

I find, however, that these undesirable characteristics of a chromium-nickel alloy of the above type may be eliminated or modified to a sufficient degree to make possible its use in dentures by incorporating therein small proportions 35 of beryllium, say from 0.1% to 5% by weight. While such additions do not affect the highly desirable corrosion resisting characteristics inherent in the chromium-nickel base alloy, they do appreciably lower its melting point, 40 increase its fluidity at casting temperatures to such an extent that extremely attenuated sections may be readily cast, and improve the surface of the casting to such a degree that a very light polishing is all that is required to complete 45 the article. Moreover, the hardness of the alloy and the yield point thereof are substantially increased. In other words, by the addition of beryllium it is possible to make an otherwise totally unsuited alloy extremely well adapted for 50 dentures.

In making my alloy the nickel and chromium are first melted together, and the beryllium, which has a very low specific gravity and is readily oxidizable, is thereafter added. Due to the 55

- lightness of the beryllium, it should be prealloyed with a suitable heavier metal, such as nickel or copper, and the addition made by tying the nickel-beryllium or copper-beryllium to a rod and plunging it into the molten mass. Once the nickel-beryllium or copper-beryllium is wet it alloys readily. Just before the molten mass is poured I prefer to add a small amount of calcium, say 0.05% as a deoxidizer.
- 10 My preferred composition contains nickel around 80%, and chromium around 20% with sufficient beryllium to obtain the desired results. This will generally be well under 5%, and since beryllium at the present time is quite expensive 15 the quantity employed will naturally be as small as possible. However, the presence of an extremely small quantity of beryllium is readily noticeable in its effect on the characteristics above mentioned of the alloy; as little as 1%, 20 for example, lowering the melting point as much as 120°. The effects of the beryllium, however, are more especially marked when the quantity is in excess of 2%.
- 25 In addition to effecting the essential changes in the base composition above noted, the beryllium, because of its extreme lightness, effects a very substantial reduction in the specific gravity of the composition which is another extremely

desirable feature of the alloy when used for dentures.

The term denture as used herein and in the appended claims is to be understood as including inlays, crowns, plates, clasps and other structures intended for use in the mouth, and also prosthetic articles in general. 5

What I claim is:

1. A denture formed from an alloy having nickel and chromium as its principal alloying ingredients and containing nickel from 65% to 90%, chromium from 5% to 30% and beryllium from 0.1% to 5%. 10

2. A cast denture formed from an alloy having nickel and chromium as its principal alloying ingredients and containing nickel from 65% to 90%, chromium from 5% to 30% and beryllium from 0.1% to 5%. 15

3. A denture formed from an alloy having nickel and chromium as its principal alloying ingredients and containing nickel from 75% to 85%, chromium from 15% to 25% and beryllium from 0.1% to 5%. 20

4. A cast denture formed from an alloy having nickel and chromium as its principal alloying ingredients and containing nickel from 75% to 85%, chromium from 15% to 25% and beryllium from 0.1% to 5%. 25

ENRIQUE G. TOUCEDA.